

[54] **PROCESS FOR THE PRODUCTION OF TECHNICAL ENDLESS FILAMENTS OF HIGH-MOLECULAR WEIGHT LINEAR POLYMERS**

[75] Inventor: **Karlheinz Riggert, Oberstedten/Ts., Germany**

[73] Assignee: **Vickers-Zimmer Aktiengesellschaft, Planung und Bau von Industrienlagen, Frankfurt, Germany**

[22] Filed: **July 24, 1970**

[21] Appl. No.: **58,054**

[30] **Foreign Application Priority Data**

Dec. 22, 1969 Germany ..... P 19 64 051.8

[52] U.S. Cl. .... **264/176 F, 264/169**

[51] Int. Cl. .... **B28b 3/20**

[58] **Field of Search** ..... **264/176 F, 169; 18/85 E, 8 SF, 8 P, 125 E, 125 B; 425/207**

[56] **References Cited**

UNITED STATES PATENTS

- |           |         |                      |           |
|-----------|---------|----------------------|-----------|
| 3,171,160 | 3/1965  | Moyer.....           | 425/207   |
| 3,480,997 | 12/1969 | List.....            | 425/207   |
| 3,104,419 | 9/1963  | LaForge .....        | 18/8 SF   |
| 3,197,533 | 7/1965  | Robinson et al. .... | 264/176 R |
| 3,479,692 | 11/1969 | Biggelaar.....       | 18/8 SF   |
| 3,506,753 | 4/1970  | Flammand.....        | 264/176 F |

|           |         |                       |           |
|-----------|---------|-----------------------|-----------|
| 3,524,221 | 8/1970  | Jones.....            | 18/8 SF   |
| 2,262,989 | 11/1941 | Conklin et al. ....   | 264/175   |
| 3,130,448 | 4/1964  | Tomlinson.....        | 264/176 F |
| 3,360,597 | 12/1967 | Jones et al. ....     | 264/176 F |
| 2,469,999 | 5/1949  | Stober .....          | 264/176 F |
| 3,437,725 | 4/1969  | Pierce.....           | 264/176 F |
| 3,457,342 | 7/1969  | Parr et al. ....      | 264/171   |
| 3,480,706 | 11/1969 | Carpenter et al. .... | 264/171   |
| 3,499,952 | 3/1970  | Koliner et al. ....   | 264/171   |

**FOREIGN PATENTS OR APPLICATIONS**

618,663 3/1961 Italy..... 264/176 F

*Primary Examiner*—Jay H. Woo

*Attorney*—Molinare, Allegretti, Newitt and Witcoff

[57] **ABSTRACT**

Process for production of endless filaments from high molecular weight polymers having improved properties of low  $\eta_{intr}$  loss, and few capillary breaks per 10 Km, in a melt spinning process wherein the polymer melt is supplied to a spinning beam at high pressure, the melt is thereafter passed through a flow path constriction which effects a pressure drop of from 150 to 1200 atmospheres and a melt enthalpy increase sufficient to internally heat each of the melt particles uniformly and independently of their position in the melt flow cross section, and thereafter maintaining the increased temperature of the melt by heating all the surfaces thereafter contacted by the melt.

8 Claims, 2 Drawing Figures



Patented Sept. 11, 1973

3,758,658



Fig. 1



Fig. 2

INVENTOR.  
Karlheinz Riggert  
BY  
Molinare, Allegretti, Newitt  
& Witcoff

**PROCESS FOR THE PRODUCTION OF  
TECHNICAL ENDLESS FILAMENTS OF  
HIGH-MOLECULAR WEIGHT LINEAR  
POLYMERS**

**BACKGROUND OF THE INVENTION**

The invention relates to a process for the production of so-called "technical" filaments and threads (yarns) of high-molecular weight linear polymers, in particular polyesters, according to an improved melt-spinning process.

An important area of use of such technical endless filaments is the production of tire cord. A number of high polymers are well suited for this utility, especially polyesters, polyamides, and their well known modifications. Such high polymers behave similarly with respect to the considerations with which this invention is concerned, i.e., at spinning temperature these polymers tend either to a state of decomposition or to after-polymerization. The processing of any high polymers exhibiting such tendencies into technical endless filaments therefore lies generally within the scope of the present invention, although in the following description reference will be made particularly to filaments of polyethylene terephthalate.

Since tire cord and the inlays formed of it are among the essential construction elements for the safety and useful life of a tire, high quality requirements are naturally placed on such endless filaments. In view of the alternating stretching and compression stresses which tires in operation experience, a necessary precondition for the use of synthetic filaments for tire cord is an adequate fatigue resistance of the filaments. As is well known, the fatigue resistance increases with the mean molecular weight of the polymer. From this, it is desirable to produce filaments with as high as possible molecular weight.

Polyethylene terephthalate has come into strong prominence in the last few years for use in tire cord production. Polyethylene terephthalate unfortunately undergoes a considerable thermal decomposition between the conclusion of the production of the spinning raw material (raw polymer melt) and its subsequent shaping into threads. This thermal decomposition increases appreciably as the molar weight of the spinning raw material rises, and — in the case of filament formation from polymer chips — cannot be prevented even by an intensive drying of the spinning raw material. Because of the thermal decomposition problem, the increase in the molecular weight of the spinning raw material which is entirely possible with polymer-forming processes of today can only in part be passed on to the spun filaments or thread formed therefrom. This thermal decomposition can be reduced, to be sure, if the molten spinning raw material is maintained for as short a time and as low a temperature as possible. However, the residence time of the spinning melt in the spinning apparatus is unfortunately prescribed by the dimensions of the apparatus, and the lower limit of the spinning temperature is determined by the highly undesirable condition of melt fracture. Where melt fracture occurs, the spun, unstretched filaments do not have a smooth or even surface, and exhibit fluctuations in diameter which are unacceptable for use as technical yarn, like tire cord.

It is evident from this that the spinning requirements are diametrically opposed. On the one hand, low melt-

ing temperature is required in the interest of a low decomposition, and on the other hand, high spinning temperature is required for trouble-free spinning. The solution of these problems was attempted by the proposal 5 described in German published application 1,292,306. There the melt was supplied at a temperature below the spinning temperature, and then the melt was heated to the spinning temperature before the filament formation. This was sought to be achieved by an arrangement 10 in which the heating box of the melt-spinning device is subdivided into two heating sections by a partition provided between the spinning pump block and the spinning head, with the heating medium being separately supplied to each section. To be sure, this proposal permits in theory separate, differentiated temperature conduction within the spinning apparatus. However, due to the relatively short residence time of the melt in the higher temperature zone and the unavoidable laminarity of flow of the highly viscous melt, the melt is not uniformly heated to the spinning temperature over the flow cross section. The undesirable consequence is inhomogeneity of the filaments over the cross section of the spinning nozzle plate, especially where the nozzle plate has a relatively large number of holes.

25 It is among the objects of the present invention to avoid these disadvantages, and in particular, to attain a rapid, uniform heating of the melt over the flow cross section before the spinning. In general terms, it is another object of the present invention to keep the loss 30 of the high molecular weight achieved by a progressive polymer-formation process as low as possible in the case of rapidly decomposing high polymers. It is another object to pass the high molecular weight on to the filaments without spinning difficulties, or in the case of 35 strongly after-polymerizing high polymers, to keep the rise in the molecular weight as low as possible.

The process of the invention solves the above problems by heating the melt prior to spinning by pressure 40 decrease by means of a flow path construction, and then maintaining the melt temperature level by corresponding heating of all the surfaces touched by the melt before the final spinning.

The process of this invention results in an ideally uniform temperature increase over the full flow cross section by energy transformation at the choke point during the pressure decrease, in which each melt particle undergoes an equally great enthalpy increase, or "tempering," independently of its position in the flow cross section. According to the invention it is assured that this 45 "tempering" state cannot be lost through heat lead-off by providing a simultaneous, corresponding heating of the spinning apparatus surfaces contacted by the melt. Characteristic of this invention is that heating by means of an external heat supply is obviated. In other words, what is characteristic of this invention is the utilization 50 of an energy transformation for the direct, brief, and uniform internal heating of the melt, in which the amount of heat required for that purpose arises within the melt itself. This requires a higher spinning pump pressure to establish the required pressure gradient, which is built up and absorbed without difficulty by a suitable dimensioning of the spinning apparatus. In the process according to this invention about a 4° C. temperature increase per 100 atmospheres of pressure gradient is obtained in the spinning processing of polyethylene terephthalate.

The threads of yarns produced according to the invention consist of filaments which are distinguished by a low scatter of both the diameter and the double refraction as measured over the thread cross section, i.e., low variation in these values from filament to filament. As a result, further processing properties are excellent. Thus, by means of a one-stage or several-stage stretching process, there can be achieved yarns or threads of high tensile strength having a low filament capillary breakage number. Furthermore, the filaments show only a relatively slight decrease in the molecular weight as compared to the spinning raw material.

In the production of technical endless filaments of polyethylene terephthalate, it has been found especially advantageous if the following conditions are met: 1) the high molecular weight melt is supplied at a temperature  $T_1$  between 280° and 330° C., and 2) is exposed to a pressure drop or pressure gradient,  $\Delta p$ , between 150 and 1200 atmospheres, at the earliest after 50 percent of its residence time between melt generation and spinning, and 3) the surface temperature,  $T_2$ , of all the surfaces contacted by the melt after the pressure drop is maintained within the following limits:

$$\frac{T_1^2}{T_1 - [17 \times 10^{-3} \Delta p]} \leq T_2 \leq \frac{T_1^2}{T_1 - \left[ 10 \left( \frac{\Delta p}{100} \right)^{2/3} \right]}$$

As the above limit formulas make clear,  $T_2$  depends on the height of the pressure gradient (drop) and the temperature  $T_1$  of the melt before the pressure drop. Preferably, the polyethylene terephthalate melt is supplied at a temperature  $T_1$  between 285° and 310° C., and is exposed to a pressure drop (gradient)  $\Delta p$  between 200 and 800 atmospheres.

It is advantageous if the pressure decrease is carried out in the flow path between spinning pump and spinning nozzle plate. Good results are achieved in the finished filaments or threads especially when the pressure drop is located in the vicinity of the spinning nozzle plate. An especially simple and effective manner of carrying out the process of this invention is in providing that the pressure drop takes place substantially at the spinning filter, which in spinning devices in general is placed in the upper part of the so-called spinning nozzle pack. Metal sieves having 10,000 to 50,000 meshes/cm<sup>2</sup> are well suited as spinning filter material for this purpose. Such sieves can be stratified in several layers one over another and are suitably supported against the high spinning pump pressure. Sintered metal filters have also proved usable for this purpose.

In principle, the pressure decrease can be carried out according to three methods or combinations thereof in the spinning apparatus. Besides the use of spinning filter as the main choke zone for achieving the pressure drop, there can be used secondly, if need be, also the filter supporting plate, or, third, the nozzle plate bores. In the case of the supporting plate and/or nozzle bores, bores with a large length/diameter ratio,  $1/d$ , are required to achieve the pressure drop required in this invention. However, unlimited  $1/d$  ratios are not possible, at least for the nozzle bores, principally for reasons of manufacturing technology. For example, diameters of less than 1mm, very common for this spinning technology, cannot be manufactured with adequate precision

where the  $1/d$  ratio is above 20. In addition, large  $1/d$  ratios are expensive to manufacture. Therefore, according to the process of this invention, the pressure is brought down preferably and largely at the spinning filter. Letting pressure down at the spinning filter is also preferable because there the temperature distribution in the melt is more uniform.

In the execution of the process of the invention, it is possible to proceed both from polymer chips, which, in 10 a known manner, are melted up on grids or by means of extruder devices, and also directly from a polymer melt obtained directly after the conclusion of the polymerization or polycondensation. In either case, short feed paths between melt discharge and spinning device 15 are recommended. The process of the invention is particularly adapted to the processing of polymers having spinning melt solution viscosities,  $\omega_{inr.}$ , equal or greater than 0.85, and preferably equal to or greater than 0.92.

20 In the drawings there is shown a spinning apparatus example suited for the process of the invention, in two schematic representations.

FIG. 1 represents a section through a spinning position of a spinning beam.

25 FIG. 2 shows a six-position beam in a rear view.

Referring now to FIG. 1, within the self-supporting and thermally insulating beam body 1 (which is cross-hatched), there are provided for each spinning position a high-pressure spinning pump 2, normally a gear wheel 30 type metering pump, having product inlet line 3 and product outlet line 4, as well as a spinning head, generally designated as 5. The spinning head 5, in the present example, being substantially rotationally symmetrical, consists of a feed plate 6 and a spinning nozzle pack 35 holder 7 screwed together with it from above (not shown). The feed plate 6 has a radially-outward directed product inlet line 8 aligned with the product outlet line 4, which product inlet line 8 expands conically downward to about the diameter of the spinning nozzle pack. The spinning nozzle pack comprises:

a. the spinning nozzle plate 9 provided with a large number of nozzle bores, which plate is seated on an inwardly-directed ring shoulder 10 of the holder 7, b. a filter support plate 11 resting on the plate 9, and c. the filter 12 sandwiched between supporting plate 11 and feed plate 6. The filter in this embodiment consists of a plurality of edge-framed wire gauze layers. The filter 12 has a double function: On the one hand it filters the spinning melt in a known manner, and on the other hand, with respect to its flow resistance, it is dimensioned in such a way that it brings about the main proportion of the desired pressure drop.

The spinning pump 2 is surrounded by a heating jacket 13, which is heated by any convenient heat transfer medium, for example the mixture of diphenyl and diphenyl oxide, while the spinning head 5 is arranged separately within its own heat transfer medium in heating vessel 14. The heating systems 13 and 14 are 55 maintained at different temperatures, so that heating jacket 13 brings about in the supplied melt the temperature  $T_1$  and heating vessel 14 maintains the temperature  $T_2$ .

As FIG. 1 makes clear, the spinning head 5 is inserted 60 from above in a receiving tube 15 of the heating vessel 14 and pressed tightly by a radially acting pressure screw 16 against the product outlet line 4. The receiving tube 15 is closed by an insulating plug 17. Prefera-

bly, the heating jacket 13 and the heating vessel 14 are each continuous for all the spinning positions of a beam, or alternatively may be constructed to communicate with one another by means of pipelines.

It should be noted that an air gap 25, 26 surrounds the spinning head 5 between it and the receiving tube 15, and the only contact point therebetween is at the radial shoulder 27, 28. The gap may range from about 1 to 3mm in width, to ensure even heat transfer from vessel 14 to the head by radiation and convection.

FIG. 2 shows that the product lines 19 are adapted to have equal length between a central supply place 18 and the individual spinning pumps 2, so that the melt has a uniform residence time for all the spinning positions. The reference number 20 designates the spinning pump drive shafts.

The process of the invention is explained in detail in the following with the aid of seven examples, of which the Example 1 describes a conventional technique not according to this invention, operating without appreciable pressure drop and without temperature rise before the spinning.

Examples 2, 5 and 7 relate to the process of this invention and clearly show its advantages.

Examples 3, 4 and 6 relate to processes in which not all the features of this invention are present simultaneously, or the work is done according to the state of technology. The solution viscosity is given in the examples as the measure for the mean molecular weight, which was determined as the  $\omega_{intr.}$  value by standard procedures. The concentration of the measuring solution amounted to 0.5 g/100 ml., the solvent is a phenol-tetrachloroethane mixture (60 : 40) and the measuring temperature was 25° C. In the examples, the diameter fluctuations along an unstretched thread filament serve as the measure of the melt fracture. The diameter fluctuations are recorded as the variation coefficient (CV<sub>D</sub> value) in percentages. In some examples also the variation coefficient of the double refraction (CV<sub>N</sub> value) is given in percentages.

#### EXAMPLE I (Conventional Technique)

A: A melt of polyethylene terephthalate having a solution viscosity of  $\omega_{intr.} = 1.04$  was supplied at a temperature T<sub>1</sub> of 310° C. to a six-position spinning beam. All the product lines, including spinning pump and spinning nozzle pack, were heated to T<sub>2</sub> = 310° C. The pressure drop in the spinning nozzle filter amounted to 80 atmospheres. From a spinning nozzle plate having 200 holes, each of 0.4 mm diameter, there was generated a thread with a spinning denier of 5900 den. at a draw-off speed of 400 m/min. The solidification of the spun thread was delayed in known manner by an after-heater, in order to preclude any undesirably great molecular pre-orientation. The mean CV<sub>D</sub> value of the unstretched thread filaments was found to be 4.8 percent, which indicates a spinning free of melt-fracture. After stretching the resultant cord base thread in a ratio of 1 : 6.1, there was found to be 20 capillary breaks per 10,000 meters and a tensile strength of 9.0 g/den. Of great disadvantage was the severe drop of the solution viscosity of the thread, which was found to be  $\omega_{intr.} = 0.86$ . B. In an otherwise corresponding test where the melt temperature was 282° C. instead of 310° C., the thread material obtained was no longer faultlessly spinnable and stretchable because of setting in of melt

fracture. In this case, the mean CV<sub>D</sub> value of the thread filaments rose to 17 percent, while the solution viscosity in the thread was  $\omega_{intr.} = 0.95$ .

#### EXAMPLE 2

(The Invention)

The initial procedure as in Example 1 was followed, but with the modification that the polymer was supplied to the spinning beam, at T<sub>1</sub> = 292° C. instead of at 310° C. The spinning beam, including spinning pump, was likewise heated to T<sub>1</sub> = 292° C. The melt residence time during its conveyance from the place of generation to the spinning beam was the same as in Example 1. In contrast to Example 1, the spinning nozzle pack was heated to a temperature of T<sub>2</sub> = 310° C. By use of a spinning nozzle filter consisting of a sieve filter combination of 24 metal screen layers each having 17,000 meshes/cm<sup>2</sup>, the pressure drop,  $\Delta p$ , was 320 atmospheres. The temperature of the spinning nozzle pack was therefore within the temperature range according to the invention. Using the spinning nozzle plate described in Example 1, a thread having spinning titer of 5900 denier was spun, again at 400 m/min. draw-off speed. The mean CV<sub>D</sub> value of the thread filaments was 4.6 percent. In agreement with Example 1, the thread had 25 breaks per 10,000 m, which is within the measurement error limits. As compared to Example 1, the molecular decomposition of the polymer was significantly improved, being considerably less under the process parameters of the invention, the thread having a solution viscosity of  $\omega_{intr.} = 0.94$ .

#### EXAMPLE 3

(Comparison)

Under the conditions of Example 2, but with a temperature T<sub>1</sub>=T<sub>2</sub> of 292° C. (lying outside the invention), a thread having a CV<sub>N</sub> value of 10 percent was obtained. The thread CV<sub>D</sub> value was 12 percent exhibiting a poor melt fracture, and the capillary break frequency of 120 breaks per 10,000 m was considerably above that of the thread of Examples 1 and 2. The  $\omega_{intr.}$  value of 0.95 showed no demonstrable advantage over that of Example 2.

#### EXAMPLE 4

(Comparison)

Initially, the same procedure as in Example 2 was followed, with the modification that the spinning nozzle pack was heated to a temperature T<sub>2</sub> of 325° C. This temperature T<sub>2</sub> lies outside the range according to this invention. The  $\omega_{intr.}$  value of the thread was 0.93 which is only a little lower than in Example 2. Although under these process conditions no melt fracture occurred, the CV<sub>D</sub> value was 10 percent, as a result of the temperature inhomogeneity of the melt emerging from the spinning nozzle plate. For the same reason, the CV<sub>N</sub> value amounted to 15 percent, and as a consequence the capillary break frequency was considerable. With respect to a thread tensile strength of 9.0 g/den. 100 capillary breaks per 10,000 m were counted.

#### EXAMPLE 5 (The Invention)

#### EXAMPLE 6 (Comparison)

#### EXAMPLE 7 (The Invention)

In the table below is presented data for three further examples. Summarized in the table are the data for the temperatures, the pressure drop, the initial and end vis-

cosities ( $\omega_{intr\ A}$  and  $\omega_{intr\ E}$ ), the viscosity decrease ( $\Delta \omega_{intr\ }$ ), the  $CV_D$  value and, in some cases the  $CV_n$  value. The advantages of working with the technique described in the present invention are easily seen by a comparison of the values for the viscosity decrease, and/or for  $CV_D$ , and/or for the capillary break numbers. For the sake of better comparison, values for Examples 1 to 4 were also included in the table.

5  
thread.

2. A process as in claim 1 wherein said polymer is a polyester.

3. A process as in claim 2 wherein:

a. said polyester is polyethylene terephthalate,  
b. said pressure drop is effected at the earliest after 50 percent of the total melt residence time between generation and spinning, and

TABLE

| Example: | $T_1$<br>(° C.) | $T_2$<br>(° C.) | $\Delta p$<br>(at) | $\eta_{intr\ A}$ | $\eta_{intr\ E}$ | $\Delta\eta_{intr.}$ | Capillary<br>break<br>number<br>for<br>10 Km. | $CV_{D_1}$<br>percent | $CV_n$<br>percent | Corresponding state of technology       |
|----------|-----------------|-----------------|--------------------|------------------|------------------|----------------------|-----------------------------------------------|-----------------------|-------------------|-----------------------------------------|
|          |                 |                 |                    |                  |                  |                      |                                               |                       |                   |                                         |
| 1a.      | 310             | 310             | 80                 | 1.04             | 0.86             | 0.18                 | 20                                            | 4.8                   | -----             | Prior art.                              |
| 1b.      | 282             | 282             | 80                 | 1.04             | 0.95             | 0.09                 | -----                                         | 17.0                  | -----             | Do.                                     |
| 2.       | 292             | 310             | 320                | 1.04             | 0.94             | 0.10                 | 25                                            | 4.6                   | 6.8               | The invention.                          |
| 3.       | 292             | 292             | 320                | 1.04             | 0.95             | 0.09                 | 120                                           | 12.0                  | 10.0              | Process not according to the invention. |
| 4.       | 292             | 325             | 320                | 1.04             | 0.93             | 0.11                 | 100                                           | 10.0                  | 15.0              | Do.                                     |
| 5.       | 285             | 322             | 760                | 0.96             | 0.87             | 0.09                 | 22                                            | 4.7                   | 7.2               | The invention.                          |
| 6.       | 285             | 285             | 120                | 0.96             | 0.89             | 0.07                 | -----                                         | 16.0                  | -----             | Process not according to the invention. |
| 7.       | 300             | 310             | 230                | 1.08             | 0.95             | 0.12                 | 27                                            | 4.5                   | 7.0               | The invention.                          |

<sup>1</sup> Melt fracture not perfectly spinnable and stretchable.

What is claimed is:

1. In a process for the production of industrial monofilaments from high-molecular weight thermoplastic polymers selected from linear polyester and polyamide polymers by melt-spinning, which high polymers are subject to decomposition or after-polymerization at spinning temperatures, including the steps of supplying a melt of said polymer at a temperature below the spinning temperature, and heating the melt prior to the filament formation, the improvement which comprises:

- a. supplying said melt at a temperature  $T_1$ , between 280° and 330° C and at high pressure to a spinning unit comprising a spinning pump, a nozzle plate and construction means disposed between said pump and said nozzle plate,  
b. passing said melt by means of said spinning pump through a constriction in its flow path said constriction occurring within said constricting means prior to said melt passing through said spinning nozzle plate to effect a pressure drop,  $\Delta p$ , of between 150 and 1200 atmospheres before arrival of said melt at said spinning nozzle, and an increase of the internal energy sufficient to internally heat the melt to a temperature greater than  $T_1$ , which increased temperature is uniform and independent of the melt position in the flow cross section under conditions which provide low loss of intrinsic viscosity and does not change the laminarity of melt flow,  
c. supplying heat from the exterior to said spinning unit surfaces thereafter contacted by said melt in an amount only sufficient to maintain the increased temperature of said internally heated melt but insufficient to cause substantial thermal degradation or after polymerization, and  
d. spinning filaments from said melt, said filaments exhibiting improved properties of low  $\omega_{intr.}$  loss, low diameter and double refraction variation coefficients, and few filament breaks per 10 Km. spun

35  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
75

3,758,658

9

c. the temperature,  $T_2$ , of all of said surfaces touched by said melt after said pressure drop is maintained within the following limits:

10

$$\frac{T_1^2}{T_1 - [(17 \times 10^{-3})(\Delta p)]} \leq T_2 \leq \frac{T_1^2}{T_1 - \left[ 10 \left( \frac{\Delta p}{100} \right)^{2/3} \right]}$$

\* \* \* \* \*

5

10

15

20

25

30

35

40

45

50

55

60

65